

Apr. 10, 1923.

1,450,935

J. L. ANDERSON

PERMANENT JOINT IN FABRICATED FORM AND METHOD OF MAKING THE SAME

Filed Dec. 12, 1918

2 sheets-sheet 1



INVENTOR

James L. Anderson  
BY  
J. P. Bauderang  
ATTORNEY

Apr. 10, 1923.

1,450,935

J. L. ANDERSON

PERMANENT JOINT IN FABRICATED FORM AND METHOD OF MAKING THE SAME

Filed Dec. 12, 1918

2 sheets - sheet 2

FIG. 3.



FIG. 4.



FIG. 2.



INVENTOR

James L. Anderson

BY  
J. F. Haubdeker

ATTORNEY

Patented Apr. 10, 1923.

1,450,935

## UNITED STATES PATENT OFFICE.

JAMES L. ANDERSON, OF BAYONNE, NEW JERSEY, ASSIGNOR, BY MESNE ASSIGNMENTS, TO AIR REDUCTION COMPANY, INCORPORATED, OF NEW YORK, N. Y., A CORPORATION OF NEW YORK.

### PERMANENT JOINT IN FABRICATED FORM AND METHOD OF MAKING THE SAME.

Application filed December 12, 1918. Serial No. 266,407.

To all whom it may concern:

Be it known that I, JAMES L. ANDERSON, a citizen of the United States, and resident of Bayonne, in the county of Hudson and State of New Jersey, have invented new and useful Improvements in Permanent Joints in Fabricated Forms and Methods of Making the Same, of which the following is a specification.

10 The object of the invention is to enable plates and other fabricated forms, of steel or other ductile metal, to be united integrally, without difficulty in the process due to expansion or contraction, and without the 15 existence of strains in the completed work likely to result in after rupture either in or out of the weld. The invention makes it possible, for example, to weld ship plates successfully, and is equally applicable in 20 other cases. The preferred manner of practising the invention will now be briefly described, with illustrations of certain of its applications.

In the drawings:

25 Figure 1 is a plan or elevation showing portions of a number of adjoining plates and illustrating various stages of the process of uniting them;

30 Fig. 2 is a cross-section through the completed weld;

Fig. 3 illustrates the application of the invention to uniting the ends of cylindrical tubular sections; and

35 Fig. 4 illustrates its application to the longitudinal seam of a tubular section or body.

In Fig. 1 rectangular plates  $a$ ,  $a^1$ ,  $a^2$ ,  $a^3$  are to be united at their edges, withoutlapping and without riveting. They may form 40 part of the outer fabric of a ship or of some other structure, and may be either flat or curved. In accordance with the invention the edges of the plates, instead of being straight, are provided with interfitting formations, especially regular indentations the sides of which are inclined at angles of  $45^\circ$  to the general direction of the joint, forming series of tapering triangular projections and recesses which match 45 when the plates are juxtaposed in predetermined manner, to form a saw-toothed seam composed of alternating reverse diagonals crossing the neutral or median general direction line. The edges are also beveled at

approximately  $45^\circ$  to the surface, so that 55 when the plates are put together a zig-zag trough is formed.

The joint between two plates, for example  $a^1$  and  $a^2$ , is fused, with an oxyacetylene or other blowpipe flame or with the electric arc, with addition of metal, at some selected spot  $b$ , so that the seam is tacked. The spot would be substantially midway of one of the diagonal sections of the indented seam, and its extent lengthwise of the seam 60 should be approximately as great as the width of the trough at the top. The seam may be regarded as composed of alternating right-hand and left-hand slopes or diagonals, forming the sides of the projections 65 or recesses. The spot  $b$  is illustrated as located upon one of the right-hand sides. At the same time that the seam is being tacked at this point, or subsequently, and before it is tacked upon another corresponding side, 70 it is fused at a spot  $b^1$ , midway of a left-hand side. The two tackings may be near together or far apart, depending upon working conditions. Thereafter the remaining 75 sides or slopes are similarly tacked at intermediate points, this stage being illustrated in the portion of the seam between the plates  $a^1$  and  $a^3$ . The first two tack welds being at reverse sides, their contraction 80 stresses oppose each other and the distortion or displacement effects are therefore neutralized. The subsequent tackings may also be performed in such order as to balance, but this is not as important as with the first 85 tackings. If desired, the seam could be tacked simultaneously at more than two points in the first instance, the locations being 90 such as to balance.

The seam has now been tacked upon opposite sides of each projection, or in other words, where the diagonals cross the neutral or center line of the seam. As indicated by dotted lines  $x$ , this leaves in both edges relatively narrow free tongues  $d$  opposed by relatively wide areas  $e$  across the seam. Upon now welding the bent or V-shaped seam-section included between two of the tack welds, this section of the weld, being of large extent relatively to the tongue, becomes, as it were, assimilated to the area  $e$  and the contraction strains are thrown largely upon the tongue  $d$ , which being 100 ductile is capable of elongation. The same

is true in respect to the welding of all these sections. In this way rupture of the weld while setting, or subsequently, due to contraction strains, is avoided, these strains being taken by the ductile tongues alternately at opposite sides of the neutral line of the seam. Owing to the form of the joint and the manner in which the weld is effected, the contraction strains taken from the weld and applied to the original metal never exceed or dangerously approach the limit of tensile strength of the metal, as may be the case with other procedures. By the multiple diagonal zigzag weld the stresses that are produced are so varied that there is no possibility of a concentration of stress in any one direction, which would be troublesome. Finally, as will now appear the remaining stresses can be relieved by reheating, without subjecting other portions of the weld to compression stresses, which in turn would become tension stresses when cool.

In order further to relieve the weld of contraction while setting, that is to say the angular sections between the tackings, it is desirable to reheat the body of the metal by the flame or otherwise opposite the sections, approximately at the regions enclosed by the dotted lines  $y$ . This urges the metal toward the weld and protects the same until it has become permanent.

A complete joint is indicated between the plates  $a^2$ ,  $a^3$ , and in section in Fig. 2. The actual melting of the bottom and sides of the trough and the manipulation of the molten metal will follow accepted autogenous or electric welding practice. The weld is filled in the regular manner by adding similar or dissimilar metal from a rod held in the blowpipe flame, in the case of flame welding, or from a rod held in the arc, if the seam is welded electrically, or from the material of the electrode itself. The finished joint is not only substantially relieved of contraction strains, but is also stronger for all purposes than a straight joint, being composed of multiple diagonal sections running in both directions. Effectively, such a weld is stronger than the original metal.

Making permanent joints in other fabricated forms does not differ materially from the case of plates. Figs. 3 and 4 show joints in readiness for welding.

The method may be used with advantage for uniting either similar or dissimilar metals.

What I claim as new is:

1. The method of obtaining permanent butt joints in fabricated forms, which comprises providing the parts to be united with interfitting indented edges consisting of tapering, substantially triangular projections and alternating recesses, and uniting said edges by fusion, whereby a saw-toothed welded joint is obtained consisting of mul-

tiple diagonals running in alternately angularly related directions across the neutral or center line of the seam.

2. The method of obtaining permanent butt joints in fabricated forms, which comprises providing the parts to be united with interfitting indented edges consisting of tapering, substantially triangular projections and alternating recesses the sides of which are substantially  $45^\circ$  to the general direction of the joint, and uniting said edges by fusion, whereby a saw-toothed welded joint is obtained consisting of multiple diagonals running in alternately angularly related directions across the neutral or center line of the seam.

3. The method of obtaining permanent butt joints in fabricated forms, which comprises providing the parts to be united with interfitting indented edges consisting of tapering, substantially triangular projections and alternating recesses, which when matched form a saw-toothed seam composed of diagonals running in alternately angularly related directions across the neutral or center line of the seam, tacking the matched edges by fusion substantially midway of the diagonals along the neutral or center line of the seam, and thereafter fusing the edges together throughout the remainder of their extent.

4. The method of obtaining permanent butt joints in fabricated forms, which comprises providing the parts to be united with interfitting indented edges consisting of tapering, substantially triangular projections and alternating recesses, which when matched form a saw-toothed seam composed of diagonals running in alternately angularly related directions across the neutral or center line of the seam, tacking the matched edges at two or more initial points substantially midway of reversed diagonals, so that the strains balance and the parts are held in proper relation, then tacking the other diagonals at approximately their middle points, along the neutral or center line of the seam, and finally completing the welding of the seam.

5. The method of obtaining permanent butt joints in fabricated forms, which comprises providing the edges of the parts to be united with interfitting tapering projections and recesses having diagonal sides, matching the edges, tacking the crooked seam by fusion at intermediate regions at the diagonals, and thereafter completing the welding of the seam.

6. The method of obtaining permanent butt joints in fabricated forms, which comprises providing the edges of the parts to be united with interfitting tapering projections and recesses having diagonal sides, matching the edges, tacking the crooked seam by fusion at intermediate regions of

the diagonals, thereafter welding the crooked or V-shaped seam portions between said regions, and reheating the body of the metal opposite said crooked seam portions before 5 the same have set.

7. The method of obtaining permanent butt joints in fabricated forms, which comprises providing the parts to be united with beveled and diagonally indented edges, 10 matching said edges, tacking them by fusion at the regions along the neutral or center line of the seam, and thereafter completing the welding of the seam with addition of metal.

8. In the production of a permanent butt joint between fabricated form portions, the steps which comprise juxtaposing two edges of interfitting formation to form an indented seam, tacking said seam at the 15 intermediate regions of the indentations, and thereafter welding the crooked seam sections between said regions.

9. In the production of a permanent butt joint between fabricated form portions, the 20 steps which comprise juxtaposing two edges of interfitting formation to form an indented seam, tacking said seam at the intermediate regions of the indentations, thereafter welding the crooked seam sections between 25 said regions, and reheating the body

of the metal opposite said crooked seam sections before the same have set.

10. In the production of a permanent butt joint between fabricated form portions, the steps which comprise juxtaposing two beveled 35 edges of interfitting formation to form an indented seam, fusing the seam together at the intermediate regions of the indentations, and thereafter completing the welding of the seam by fusion with addition of metal.

11. A permanent butt joint comprising indented edges composed of tapering projections and intervening recesses matched and fused together in a welded seam composed of 40 diagonals alternately reversely inclined to the neutral or center line of the seam.

12. A permanent butt joint comprising indented matched edges fused together in a substantially saw-toothed welded seam composed of 45 diagonals alternately reversely inclined at approximately 45° to the neutral or center line of the seam.

13. A fabricated structure comprising plates having saw-toothed edges interfitted and fused together, presenting a welded seam substantially all portions of which are 50 diagonal to the general direction of the seam.

JAMES L. ANDERSON.